

## UNITED STATES PATENT OFFICE

WILLOUGHBY STATHAM SMITH, OF NEWTON POPPLEFORD, AND HENRY JOSEPH GARNETT, OF SEVENOAKS, ENGLAND

## MAGNETIC ALLOY

No Drawing. Original application filed May 7, 1927, Serial No. 189,735, and in Great Britain July 27, 1926. Divided and this application filed July 17, 1928. Serial No. 293,484.

This application is a division of application, Ser. No. 189,735, filed May 7, 1927.

In the Patent No. 1,552,769, granted Sept. 8, 1925, a number of alloys with high permeability with very weak magnetizing forces were described; amongst others, alloys composed as follows:—

|           | No. 1 | No. 2 |
|-----------|-------|-------|
| Nickel    | 70.5% | 65%   |
| Iron      | 18.5% | 17%   |
| Copper    | 10.5% | 17%   |
| Manganese | 0.5%  | 0.5%  |

The first alloy had a magnetic permeability of 5300, and the second a magnetic permeability of 3200 in magnetic fields tending to zero.

According to this invention an alloy is composed of:—

|           |        |
|-----------|--------|
| 20 Nickel | 69-71% |
| Iron      | 14-15% |
| Copper    | 14-16% |

The magnetic permeability of such alloy, when suitably annealed (by heating to a temperature in excess of the magnetic change point and cooled so that its initial permeability is of the order of 6000) is almost independent of the strength of the field between  $H=.001$  and  $H=.1$  gauss. The alloy should be heated to a temperature of about 880° C. and air cooled.

For example an alloy containing substantially:—

|           |     |
|-----------|-----|
| 35 Nickel | 70% |
| Iron      | 15% |
| Copper    | 15% |

with a trace of manganese, has given the following results when drawn to fine wire, annealed and tested:—

$$\begin{aligned} H=.001 &= 6300 \\ &=.01 = 6800 \\ &=.05 = 7400 \end{aligned}$$

15 The alloy has properties, therefore, which make it, in a tape or wire form, very useful for the manufacture of loaded telegraphic and telephonic cables.

50 To the alloy may be added manganese in

quantities of less than .5% as a deoxidizer, but should not contain any trace of carbon.

What we claim is:—

1. The combination with an electrical conductor of loading material applied to said conductor and comprising iron from 14 to 15%, copper from 14 to 16%, and the remainder nickel, the initial permeability of said material being of the order of 6,000. 55

2. The combination with an electrical conductor of loading material applied to said conductor and comprising iron from 14 to 15%, copper from 14 to 16%, and the remainder nickel, said material having had an initial permeability of the order of 6,000 developed by heating to a temperature in excess of the magnetic change point and then cooling. 65

3. The combination with an electrical conductor of loading material applied to said conductor and comprising iron from 14 to 15%, copper from 14 to 16%, a deoxidizing metal to an amount not greater than 0.5%, and the remainder nickel, the initial permeability of said material being of the order 75 of 6,000.

4. The combination with an electrical conductor of loading material applied to said conductor and comprising iron from 14 to 15%, copper from 14 to 16%, a deoxidizing metal to an amount not greater than 0.5%, and the remainder nickel, said material having had an initial permeability of the order of 6,000 developed by heating to a temperature in excess of the magnetic change point 85 and then cooling.

In testimony that we claim the foregoing as our invention we have signed our names this twenty-ninth day of June, 1928.

WILLOUGHBY STATHAM SMITH. 90  
HENRY JOSEPH GARNETT.